



US009815103B2

(12) **United States Patent**  
Norita et al.

(10) Patent No.: US 9,815,103 B2  
(45) Date of Patent: Nov. 14, 2017

- (54) **WARM WORKING METHOD FOR STAINLESS STEEL FOIL AND MOLD FOR WARM WORKING**

(71) Applicant: **NISSHIN STEEL CO., LTD.**, Tokyo (JP)

(72) Inventors: **Katsunari Norita**, Osaka (JP); **Norimasa Miura**, Osaka (JP)

(73) Assignee: **Nissin Steel Co., Ltd.**, Tokyo (JP)

(\*) Notice: Subject to any disclaimer, the term of this patent is extended or adjusted under 35 U.S.C. 154(b) by 0 days.

(21) Appl. No.: **15/291,177**

(22) Filed: **Oct. 12, 2016**

(65) **Prior Publication Data**

US 2017/0028456 A1 Feb. 2, 2017

### **Related U.S. Application Data**

- (62) Division of application No. 14/431,665, filed as application No. PCT/JP2013/076028 on Sep. 26, 2013.

(30) **Foreign Application Priority Data**

Sep. 28, 2012 (JP) ..... 2012-215865  
Sep. 25, 2013 (JP) ..... 2013-198203

(51) Int. Cl.

*B21D 24/00* (2006.01)  
*B21D 24/16* (2006.01)  
*B21D 33/00* (2006.01)  
*B21D 22/20* (2006.01)  
*B21D 37/16* (2006.01)

(52) U.S. Cl.

CPC ..... **B21D 24/16** (2013.01); **B21D 22/208**  
(2013.01); **B21D 33/00** (2013.01); **B21D**  
**37/16** (2013.01)

- (58) **Field of Classification Search**  
CPC ..... B21D 33/00; B21D 22/208; C22C 38/18;  
Y10T 29/301; Y10T 29/30  
See application file for complete search history.

(56) **References Cited**

U.S. PATENT DOCUMENTS

9,257,682 B2 \* 2/2016 Norita ..... B21D 22/22

## FOREIGN PATENT DOCUMENTS

|    |            |   |         |
|----|------------|---|---------|
| CN | 102886422  | A | 1/2013  |
| CN | 103443955  | A | 12/2013 |
| JP | H05 237558 | A | 9/1993  |
| JP | H11-309519 | A | 11/1999 |
| JP | 2005205416 | A | 8/2005  |

(Continued)

## OTHER PUBLICATIONS

A communication issued in corresponding Chinese application 201380050840.2 dated Oct. 8, 2015, 6 pages.

(Continued)

*Primary Examiner* — Richard Chang

(74) *Attorney, Agent, or Firm* — Rothwell, Figg, Ernst & Manbeck P.C.

(57) **ABSTRACT**

An austenitic stainless steel foil 2 with a thickness equal to or less than 300  $\mu\text{m}$  is disposed to face a punch 12, and the stainless steel foil 2 is subjected to drawing in a state in which an annular region 2a of the stainless steel foil 2 that is in contact with a shoulder portion 12d of the punch 12 is set to a temperature up to 30° C. and an external region 2b outside the annular region 2a is set to a temperature of from 40° C. to 100° C.

## 1 Claim, 3 Drawing Sheets



(56)

**References Cited**

FOREIGN PATENT DOCUMENTS

|    |             |    |         |
|----|-------------|----|---------|
| JP | 2009-113058 | A  | 5/2009  |
| JP | 2012216511  | A  | 11/2012 |
| WO | 2012/132956 | A1 | 10/2012 |

OTHER PUBLICATIONS

Supplementary European Search Report dated May 6, 2016, for corresponding European application EP 13 84 2476, 8 pages.

\* cited by examiner

Fig. 1



Fig. 2



Fig. 3



Fig. 4



Fig. 5



Fig. 6



1

## WARM WORKING METHOD FOR STAINLESS STEEL FOIL AND MOLD FOR WARM WORKING

This application is a divisional of U.S. Ser. No. 14/431, 665 filed Mar. 26, 2015 which is a 35 U.S.C. §371 National Phase Entry Application from PCT/JP2013/076028, filed Sep. 26, 2013, and designating the United States, which claims priority under 35 U.S.C. §119 to Japanese Patent Application No. 2012-215865 filed on Sep. 28, 2012, and to Japanese Patent Application No. 2013-198203 filed on Sep. 25, 2013, which are incorporated herein by reference in their entireties.

### TECHNICAL FIELD

The present invention relates to a warm working method for stainless steel foil by which stainless steel foil is subjected to drawing, and also relates to a mold for warm working.

### BACKGROUND ART

Patent Literature 1 listed hereinbelow discloses an example of a conventional warm working method for a stainless steel foil of this type. Thus, Patent Literature 1 describes cooling a punch to 0°C. to 30°C. and heating a pressure pad to 60°C. to 150°C. when drawing an austenitic stainless steel sheet with a thickness of about 800 μm to 1000 μm.

Patent Literature 1: Japanese Patent Application Publication No. 2009-113058.

### DISCLOSURE OF THE INVENTION

The inventors have investigated the application of the drawing such as described in Patent Document 1 to a thin stainless steel foil with a thickness equal to or less than 300 μm and encountered the following problem. Namely, the method described in Patent Document 1 is for working a comparatively thick stainless steel sheet with a thickness of about 800 μm to 1000 μm, and when this method is directly applied to a thin stainless steel foil with a thickness equal to or less than 300 μm, cracks occur and deep drawing sometimes cannot be realized.

The present invention has been created to resolve this problem, and it is an objective of the present invention to provide a warm working method for a stainless steel foil that can suppress the occurrence of cracks and can realize deep drawing more reliably even in the case of a thin stainless steel foil with a thickness equal to or less than 300 μm.

The warm working method for a stainless steel foil according to the present invention includes: disposing an austenitic stainless steel foil with a thickness equal to or less than 300 μm to face a punch and subjecting the stainless steel foil to drawing in a state in which an annular region of the stainless steel foil that is in contact with a shoulder portion of the punch is set to a temperature up to 30°C. and an external region outside the annular region is set to a temperature of from 40°C. to 100°C.

A mold for warm working a stainless steel foil in accordance with the present invention includes: a punch; a blank holder disposed at an outer circumferential position of the punch; and a die disposed to face the blank holder, and serves to subject an austenitic stainless steel foil with a thickness equal to or less than 300 μm to drawing by pressing the stainless steel foil together with the punch

2

inward of the die in a state in which the stainless steel foil is interposed between the blank holder and the die, wherein the punch is provided with cooling means; the blank holder and the die are provided with heating means; and the stainless steel foil is subjected to drawing in a state in which an annular region of the stainless steel foil that is in contact with a shoulder portion of the punch is set to a temperature equal to or less than 30°C. and an external region outside the annular region interposed between the blank holder and the die is set to a temperature of from 40°C. to 100°C.

With the warm working method for a stainless steel foil in accordance with the present invention, the stainless steel foil is subjected to drawing in a state in which the annular region of the stainless steel foil that is in contact with the shoulder portion of the punch is set to a temperature equal to or less than 30°C. and an external region outside the annular region is set to a temperature of from 40°C. to 100°C. or lower. Therefore, the occurrence of cracks can be suppressed and deep drawing can be realized more reliably even in the case of a thin stainless steel foil with a thickness equal to or less than 300 μm.

### BRIEF DESCRIPTION OF THE DRAWINGS

FIG. 1 is a configuration diagram illustrating a mold for warm working that is used for implementing a warm working method for a stainless steel foil according to Embodiment 1 of the present invention.

FIG. 2 is a graph illustrating the difference in a limit drawing ratio caused by the difference in a sheet thickness.

FIG. 3 is a graph illustrating the difference in the increase of temperature caused by the difference in a sheet thickness.

FIG. 4 is a graph illustrating the difference in a tensile strength change caused by the difference in a sheet thickness.

FIG. 5 is a configuration diagram illustrating a mold for warm working that is used for implementing a warm working method for a stainless steel foil according to Embodiment 2 of the present invention.

FIG. 6 is an explanatory drawing illustrating the difference in temperature distribution of a blank holder caused by the presence of a thermally insulating plate.

### BEST MODE FOR CARRYING OUT THE INVENTION

Embodiments of the present invention are explained hereinbelow with reference to the appended drawings.

#### Embodiment 1

FIG. 1 is a configuration diagram illustrating a mold 1 for warm working that is used for implementing a warm working method for a stainless steel according to Embodiment 1 of the present invention. As depicted in the figure, the mold 1 for warm working is provided with a lower mold 10 and an upper mold 15 disposed such as to sandwich a stainless steel foil 2. The lower mold 10 is provided with a bed 11, a punch 12 fixed to the bed 11, and a blank holder 14 that is disposed at the outer circumferential position of the punch 12 and coupled to the bed 11 through a cushion pin 13. The upper mold 15 is provided with a slide 16 and a die 18 disposed above the blank holder 14 and fixed to the slide 16 through a spacer 17.

A servo motor (not shown in the figure) is connected to the slide 16. The slide 16, the spacer 17, and the die 18, that is, the upper mold 15, are driven integrally by a drive force

from the servo motor in the direction of approaching the lower mold 10 and withdrawing therefrom. After the stainless steel foil 2 has been disposed so as to face the punch 12, the upper mold 15 is shifted in the direction approaching the lower mold 10. As a result, the punch 12 is pressed into the stainless steel foil 2 and the die 18, and the stainless steel foil 2 is subjected to drawing.

The punch 12 is provided with cooling means constituted by an introduction path 12a connected to an external coolant system (not shown in the figure), a cooling chamber 12b into which a coolant is introduced through the introduction path 12a, and a discharge path 12c through which the coolant is discharged from the cooling chamber 12b. Thus, the punch 12 can be cooled by introducing the coolant into the cooling chamber 12b. As a result of bringing such cooled punch 12 into contact with the stainless steel foil 2, the annular region 2a of the stainless steel foil 2 which is in contact with a shoulder portion 12d of the punch 12 is cooled. The cooling range of the stainless steel foil 2 may include at least the annular region 2a, but may include not only the annular region 2a, but also an inner region of the annular region 2a. The present embodiment is configured such that the stainless steel foil 2 is cooled by the punch 12. Therefore, not only the annular region 2a, but also the inner region of the annular region 2a is cooled.

A counter punch coupled through a spring or the like to the slide can be disposed at a position facing the punch, and a cooling chamber into which the coolant is introduced can be provided in the counter punch, thereby further increasing the cooling efficiency of the stainless steel foil 2 (this configuration is not shown in the figure).

Heaters 14a, 18a (heating means) for heating the blank holder 14 and the die 18 are incorporated in the blank holder 14 and the die 18. Since the stainless steel foil 2 is sandwiched by the heated blank holder 14 and die 18, the external region 2b of the annular region 2a is heated.

The stainless steel foil 2 is an uncoated austenitic stainless steel which is not provided with an additional layer, for example such as a resin layer, on the front or rear surface. A thin foil with a thickness equal to or less than 300  $\mu\text{m}$  is used as the stainless steel foil 2.

A warm working method for the stainless steel foil 2 performed by using the mold 1 for warm working which is depicted in FIG. 1 is described below. When the upper mold 15 is withdrawn from the lower mold 10, the stainless steel foil 2 is placed on the punch 12 and the blank holder 14 so as to face the punch 12, and the upper mold 15 is thereafter lowered to a position in which the stainless steel foil 2 is sandwiched between the blank holder 14 and the die 18. Where the punch 12 is disposed at the upper side and the die 18 is disposed at the lower side, the stainless steel foil 2 is placed on the die 18.

In this case, as a result of cooling the punch 12 and heating the blank holder 14 and the die 18, the annular region 2a of the stainless steel foil 2 is at a temperature of from 0° C. to 30° C. and the external region 2b of the stainless steel foil 2 is at a temperature of from 40° C. to 100° C., preferably from 60° C. to 80° C.

The annular region 2a is set to a temperature of up to 30° C. because where the temperature thereof is higher than 30° C., a sufficient increase in breaking strength caused by the martensitic transformation cannot be obtained. Further, the annular region 2a is set to a temperature of 0° C. or higher because where the temperature of the annular region is less than 0° C., frost adheres to the punch 12 or the annular region and moldability of the molded product is lost. In

addition, the molded article can collapse as a result of temperature-induced shrinkage at the time of removal from the mold.

The external region 2b is set to a temperature of from 40° C. because where the temperature of the external region 2b is less than 40° C., the hardening caused by the martensitic transformation cannot be sufficiently suppressed. The external region 2b is set to a temperature of up to 100° C. because where the temperature of the external region 2b is higher than 100° C., the temperature of the annular region 2a rises due to a transfer of heat from the external region 2b to the annular region 2a, and a sufficient increase in a breaking strength of the punch caused by the martensitic transformation cannot be obtained.

As indicated hereinabove, working at a larger drawing ratio (ratio of the workpiece diameter to the product diameter) can be performed by setting the temperature of the external region 2b to from 60° C. to 80° C. The temperature is set to from 60° C. because the effect of suppressing the hardening caused by the martensitic transformation can be demonstrated more reliably, and the temperature is set up to 80° C. because the temperature rise of the annular region 2a can be suppressed.

By setting the temperature of the external region 2b to from 40° C. to less than 60° C., it is possible to shorten the time required for temperature restoration of the mold 1 for warm working (time required for the temperature of the blank holder 14 and the die 18, which has decreased due to contact with the stainless steel foil 2, to return to a range of from 40° C. to less than 60° C.) and increase the working efficiency while enabling deep drawing.

After the temperatures of the annular region 2a and the external region 2b have been set to the above-described temperatures, the upper mold 15 is further lowered. As a result, the punch 12 is pressed into the stainless steel foil 2 and the die 18, drawing is implemented, and the stainless steel foil 2 is molded into a hat shape. A lubricating oil is supplied to the punch 12, the die 18, and the stainless steel foil 2 through the entire drawing process.

FIG. 2 is a graph illustrating the difference in a limit drawing ratio caused by the difference in sheet thickness. FIG. 3 is a graph illustrating the difference in the increase of temperature caused by the difference in sheet thickness. FIG. 4 is a graph illustrating the difference in a tensile strength change caused by the difference in sheet thickness.

As an example, the inventors performed drawing of the stainless steel foil 2 with a thickness of 100  $\mu\text{m}$ . As a comparative example, a stainless steel sheet with a thickness of 800  $\mu\text{m}$  was subjected to drawing. The temperature of the external region 2b (the blank holder 14 and the die 18) was changed from 40° C. to 120° C. while changing the diameter of the stainless steel foil 2 and the stainless steel sheet, and the limit drawing ratio (ratio of the workpiece diameter to the product diameter) at which no cracks occurred was examined. The diameter of the punch 12 was 40.0 mm, the punch shoulder R was 2.5 mm, the inner diameter of the die 18 was 40.4 mm, the die shoulder R was 2.0 mm, and the temperature of the annular region 2a (punch 12) was 10° C. to 20° C.

As depicted in FIG. 2, it was determined that in the case of the stainless steel foil 2 with a thickness of 100  $\mu\text{m}$ , sufficient deep drawing could be realized by setting the temperature of the external region 2b from 40° C. to 100° C. In particular, it was determined that drawing at a larger drawing ratio could be performed by setting the temperature of the external region 2b from 60° C. to 80° C.

Meanwhile, in the case of the stainless steel plate with a thickness of 800  $\mu\text{m}$ , it was necessary to set the temperature of the external region  $2b$  to from 80° C. to 160° C. in order to perform the deep drawing similar to that of the above-described stainless steel foil **2** with a thickness of 100  $\mu\text{m}$ . Thus, it was determined that the optimum working temperature of the stainless steel foil **2** with a thickness of 100  $\mu\text{m}$  had shifted to the low-temperature side with respect to the optimum working temperature of the stainless steel sheet with a thickness of 800  $\mu\text{m}$ . This comparison confirmed that deep drawing cannot be realized by simple application of the method for working a stainless steel sheet with a thickness of 800  $\mu\text{m}$  to a stainless steel foil **2** with a thickness of 100  $\mu\text{m}$ .

The following reason can be suggested for explaining the shift of the optimum working temperature to the low-temperature side. Specifically, as depicted in FIG. 3, thermal conductivity of a stainless steel foil **2** with a thickness of 100  $\mu\text{m}$  is higher than that of a stainless steel sheet with a thickness of 800  $\mu\text{m}$ . In other words, in a stainless steel foil **2** with a thickness of 100  $\mu\text{m}$ , the heat of the external region  $2b$  is easier transferred to the annular region  $2a$ . Therefore, where the temperature of the external region  $2b$  in a stainless steel foil **2** with a thickness of 100  $\mu\text{m}$  becomes too high, the temperature of the annular region  $2a$  increases and a sufficient increase in the breaking strength caused by the martensitic transformation cannot be obtained. As a consequence, the workability of a stainless steel foil **2** with a thickness of 100  $\mu\text{m}$  is degraded unless the temperature is lower than that of the stainless steel sheet with a thickness of 800  $\mu\text{m}$ , which is apparently why the optimum working temperature shifts to a low-temperature side.

Further, where the tensile strength change of a stainless steel foil **2** depicted in FIG. 4 is compared with that of a stainless steel sheet, it can be found that the tensile strength change in a low-temperature region of the stainless steel foil is higher. Therefore, in the case of a stainless steel foil **2** with a thickness of 100  $\mu\text{m}$ , a difference in strength similar to that in a stainless steel sheet with a thickness of 800  $\mu\text{m}$  can be obtained at a heating amount which is half or less than that in the case of a stainless steel sheet with a thickness of 800  $\mu\text{m}$ . Thus, since a stainless steel foil **2** with a thickness of 100  $\mu\text{m}$  can be softened at a temperature lower than that of a stainless steel sheet with a thickness of 800  $\mu\text{m}$ , the optimum working temperature shifts to a low-temperature side.

In the explanation using FIGS. 2 and 3, a stainless steel foil **2** with a thickness of 100  $\mu\text{m}$  is considered, but sufficient deep drawing can be realized in the same temperature region with any stainless steel foil **2** with a thickness equal to or less than 300  $\mu\text{m}$ . This is because in a stainless steel foil **2** with a thickness equal to or less than 300  $\mu\text{m}$ , the degree of thermal effect produced on the tensile strength change demonstrates the same trend as in a stainless steel foil **2** with a thickness of 100  $\mu\text{m}$ . Sufficient deep drawing can also be realized in the same temperature region even with a very thin stainless steel foil **2** with a thickness equal to or less than 5  $\mu\text{m}$ , provided that such foil can be worked with the mold **1** for warm working.

With such a warm working method and mold **1** for warm working of a stainless steel foil **2**, a stainless steel foil **2** is subjected to drawing in a state in which the annular region  $2a$  of the stainless steel foil **2** that is in contact with the shoulder portion  $12d$  of the punch **12** is set to a temperature up to 30° C. and the external region  $2b$  of the annular region  $2a$  is set to a temperature of from 40° C. to 100° C. Therefore, the occurrence of cracking can be suppressed and deep drawing can be realized more reliably even with

respect to a thin stainless steel foil with a thickness equal to or less than 300  $\mu\text{m}$ . Such a warm working method is particularly useful, for example, for the production of containers such as battery covers that have to combine high strength with reduced weight.

Further, where the temperature of the external region  $2b$  is set to from 60° C. to 80° C. when the stainless steel foil **2** is subjected to drawing, the working can be performed at a higher drawing ratio.

Furthermore, where the temperature of the external region  $2b$  is set to from 40° C. to less than 60° C. when the stainless steel foil **2** is subjected to drawing, it is possible to shorten the time required for temperature restoration of the mold **1** for warm working and increase the working efficiency while realizing deep drawing.

## Embodiment 2

FIG. 5 is a configuration diagram illustrating the mold **1** for warm working that is used for implementing a warm working method for a stainless steel foil according to Embodiment 2 of the present invention. As depicted in FIG. 5, in the mold **1** for warm working according to Embodiment 2, a thermally insulating plate **19** (thermally insulating member) constituted by glass fibers as a main base material and a borate binder as a main material is provided at the inner circumferential portion of the blank holder **14** facing the outer circumferential surface of the punch **12**. Other features are the same as in Embodiment 1.

FIG. 6 is an explanatory drawing illustrating the difference in temperature distribution of the blank holder **14** caused by the presence of the thermally insulating plate **19**. Thus, FIG. 6(a) depicts the temperature distribution obtained when the thermally insulating plate **19** is not provided, and FIG. 6(b) depicts the temperature distribution obtained when the thermally insulating plate **19** is provided. FIGS. 6(a) and 6(b) each represent the results obtained by measuring the surface temperature of the blank holder **14** with a contact thermometer after the blank holder was allowed to stay for 30 min at a set temperature of 70° C.

In the configuration which is not provided with the thermally insulating plate **19**, as depicted in FIG. 6(a), the deviation of the surface temperature of the blank holder **14** reaches 30° C. at maximum. A low temperature in the upper portion depicted in the figure is due to the presence of a lead-out portion of a control thermocouple or heater **14a** in this portion. Meanwhile, in the configuration which is provided with the thermally insulating plate **19** at the inner circumferential portion of blank holder **14**, as depicted in FIG. 6(b), the temperature distribution is greatly reduced. This is apparently because the presence of the thermally insulating plate **19** at the inner circumferential portion prevents the heat of the heater **14a** from escaping to the central hole (hole for inserting the punch **12**) of the blank holder **14** and the heat of the heater **14a** spreads uniformly over the entire blank holder **14**. This temperature distribution indicates that the heat of the blank holder **14** is unlikely to be transferred to the punch **12** due to the presence of the thermally insulating plate **19** at the inner circumferential portion of the blank holder **14**.

An example is explained hereinbelow. The inventors continuously implemented at 30-sec intervals the drawing of stainless steel foils **2** with a thickness of 100  $\mu\text{m}$  by using the mold **1** for warm working (with the thermally insulated structure) depicted in FIG. 5 and the mold **1** for warm working (without a thermally insulated structure) depicted in FIG. 1. In the continuous drawing, the set temperature of the

external region **2b** (blank holder **14** and die **18**) was 70° C. and the set temperature of the annular region **2a** (punch **12**) was 10° C. to 20° C. The possibility of continuous press working was then investigated. The results are shown in Table 1 below.

The working shape was an angular tubular shape with a molding height of 40 mm, the punch **12** had a shape of 99.64×149.64 mm, the punch shoulder R was 3.0 mm, the punch corner R was 4.82 mm, the die **18** had a shape of 100×150 mm, the die shoulder R was 3.0 mm, and the die corner R was 5.0 mm.

TABLE 1

|                 | With thermally insulated structure | Without thermally insulated structure |
|-----------------|------------------------------------|---------------------------------------|
| Number of times |                                    |                                       |
| 1               | ○                                  | ○                                     |
| 2               | ○                                  | ○                                     |
| 3               | ○                                  | ○                                     |
| 4               | ○                                  | X                                     |
| 5               | ○                                  | —                                     |
| 6               | ○                                  | —                                     |
| 7               | ○                                  | —                                     |
| 8               | ○                                  | —                                     |
| 9               | ○                                  | —                                     |
| 10              | ○                                  | —                                     |

As shown in Table 1, where the results of continuous press working obtained with the mold **1** for warm working (with a thermally insulated structure) depicted in FIG. 5 and the mold **1** for warm working (without a thermally insulated structure) depicted in FIG. 1 are compared, the number of possible continuous pressing operations with the former mold is larger than that with the latter mold. This is apparently because the presence of the thermally insulating plate **19** on the inner circumferential portion of the blank holder **14** makes it possible to avoid increases in the temperature of the punch **12** caused by the heat of the blank holder **14** and maintain a more adequate relationship between the temperatures of the annular region **2a** and the

external region **2b**. When the temperature of the punch **12** was measured before and after the continuous pressing, the temperature change was less and the temperature was more stable with the mold **1** for warm working (with a thermally insulated structure) depicted in FIG. 5.

With such warm working method and mold **1** for warm working of the stainless steel foil **2**, since the thermally insulating plate **19** is provided at the inner circumferential portion of the blank holder **14**, the increase in the temperature of the punch **12** caused by the heat of the blank holder **14** can be avoided and continuous drawing can be performed more reliably in a short interval of time.

The invention claimed is:

1. A mold for warm working an austenitic stainless steel foil, the mold comprising:
  - a punch;
  - a blank holder disposed at an outer circumferential position of the punch; and
  - a die disposed to face the blank holder, and
  - wherein the mold is configured to subject the austenitic stainless steel foil with a thickness equal to or less than 300  $\mu$ m to draw by pressing the austenitic stainless steel foil together with the punch inward of the die such that the austenitic stainless steel foil is interposed between the blank holder and the die, wherein
  - the punch is provided with cooling means,
  - the blank holder and the die are provided with heating means, and
  - the austenitic stainless steel foil is subjected to draw such that an annular region of the austenitic stainless steel foil that is in contact with a shoulder portion of the punch is set to a temperature equal or up to 30° C. and an external region outside the annular region interposed between the blank holder and the die is set to a temperature from 40° C. to 100° C.,
  - wherein a thermally insulating member is provided at an inner circumferential portion of the blank holder facing an outer circumferential surface of the punch.

\* \* \* \* \*